

# United States Patent

Peterson

[15] 3,638,293

[45] Feb. 1, 1972

[54] **HIGH-DENSITY TUNGSTEN-RHENIUM-NICKEL ALLOYS AND ARTICLES**

[72] Inventor: Sven Torsten Lennart Peterson, Vendelso, Sweden

[73] Assignee: Lumalampen Aktiebolag, Stockholm, Sweden

[22] Filed: Sept. 12, 1969

[21] Appl. No.: 857,478

[52] U.S. Cl. .... 29/182, 75/176, 75/221, 252/515

[51] Int. Cl. .... B22f 3/00

[58] Field of Search.... 29/182; 75/176; 252/515

2,227,445 1/1941 Driggs..... 75/200  
2,466,992 4/1949 Kurtz..... 75/176  
3,359,082 12/1967 Dickinson..... 29/182

Primary Examiner—Carl D. Quarforth

Assistant Examiner—R. E. Schafer

Attorney—Herbert H. Goodman

[57]

## ABSTRACT

Sintered alloys of tungsten containing between about 1 percent and 7.5 percent rhenium and between about 0.15 percent and 0.3 percent nickel and electrical articles, particularly contacts, prepared from said alloys. The invention also includes a method of improving the density of tungsten alloys.

[56] References Cited

UNITED STATES PATENTS

2,157,935 5/1939 Hensel..... 75/176

14 Claims, 3 Drawing Figures





INVENTOR  
SVEN TORSTEN LENNART PETERSON

BY Bauer & Goodman

ATTORNEYS

PATENTED FEB 1 1972

3,638,293

SHEET 2 OF 2



FIG. 2



FIG. 3

## HIGH-DENSITY TUNGSTEN-RHENIUM-NICKEL ALLOYS AND ARTICLES

### BACKGROUND OF THE INVENTION

Tungsten is widely used in industry for electrical materials such as contacts. The most widely used method for manufacturing tungsten articles is the powder metallurgic method. This conventionally involves preparation of the metal powder (or mixture of metal powders when alloys are to be prepared), reduction, pressing, presintering, and then sintering to obtain a relatively dense article. Presintering and sintering are carried out in an inert or reducing atmosphere. This is usually followed by working, i.e., cold working or hot working, such as pressing, rolling, swaging, etc., to increase density. The sequence of operations depends upon the specific article being manufactured and the properties and characteristics desired. These include electrical and tensile properties, recrystallization characteristics, grain size and orientation, porosity, nonmetallic inclusions, density, purity, etc.

It is a major advantage to obtain an article in the "as sintered" condition having the greatest possible density. This eliminates further working such as swaging. The advantages that follow are lower costs and minimized effect upon the recrystallization properties. It is also advantageous to obtain maximum density or the desired density at lower sintering temperatures, and particularly temperatures not higher than about 1,500-1,600° C. This results in lower cost and the ability to utilize conventional sintering furnaces. It also avoids the undesirable effects upon the electrical and/or metallographic characteristics that sometime result from extremely high temperature sintering.

The present invention provides high density tungsten-rhenium-nickel alloys and articles made therefrom.

### BRIEF SUMMARY OF INVENTION

Sintered high-density alloy compositions containing between about 1 and 7.5 percent rhenium and between about 0.15 and 0.3 percent nickel, and electric contacts prepared therefrom.

The preferred compositions have a density of at least 18.6 g./cc. and more preferably, a density of at least 19 g./cc.

Within the range of alloys disclosed and of electrical contact alloy compositions, preferred compositions include the following: Between 2 and 7 percent rhenium and between 0.2 and 0.3 percent nickel; between 1 and 7.5 percent rhenium and 0.3 percent nickel; between 2 and 5.5 percent rhenium and 0.2 and 0.3 percent nickel; and about 3 percent rhenium and 0.15 percent nickel.

The following compositions are also useful, although not as preferred as those listed in the preceding paragraph: Between 1 and 5.5 percent rhenium and 0.15 and 0.3 percent nickel; and between 2 and 4 percent rhenium and 0.15 percent nickel.

### BRIEF DESCRIPTION OF DRAWINGS

FIG. 1 is a graph relating alloy compositions to the density "as sintered" for the conditions and compositions in the examples herein;

FIG. 2 is a photomicrograph, 100 x, of an unetched section of the "as sintered" alloy composition containing 0.2 percent nickel, 3 percent rhenium and the remainder tungsten; and

FIG. 3 is a photomicrograph, 425 x, of an etched section of the same alloy.

### DETAILED DESCRIPTION OF INVENTION

The tungsten alloy articles of the present invention are manufactured by conventional powder metallurgic techniques. The alloy powder mixture may be prepared by admixing powders of nickel, rhenium and tungsten. They are preferably prepared by admixing reducible metal compounds of each of the metals. Nickel is preferably added as nickel carbonate or nickel oxide. Rhenium is preferably added as am-

monium perrhenate. Tungsten is preferably added as tungstic oxide. Mixing is preferably carried out in a ball mill having a liquid medium, e.g., alcohol, methylene chloride, etc. After mixing has been carried out until a homogeneous mixture is attained, the mixture is removed from the ball mill, dried and reduced in hydrogen, preferably at a temperature of between about 700° and 1,000° C. The resultant mixed metal powders are preferably treated by addition of a hydrocarbon material such as paraffin wax in a solvent to improve compactability. A green compact is then formed by pressing, preferably at a pressure of about 15 tons per square inch. The green compact is then presintered, preferably at a temperature of about 800° to 1,000° C. for a period of about one-half hour. Sintering is then carried out at elevated temperatures. The preferred sintering temperature, utilizing the alloy compositions of the present invention, is between about 1,400° and 1,550° C. Sintering time is preferably between about 1 and 3 hours. This relatively low temperature sintering provides the desired density without at the same time reaching sufficiently high temperatures to undesirably affect physical and metallographic properties. Presintering and sintering are carried out in a protective atmosphere, i.e., vacuum, an inert atmosphere or a reducing atmosphere. The sintered articles may then be finished by tumbling or lapping, or, if necessary, finish machined to the desired dimensions.

The invention is further illustrated in the following examples. All parts and percentages specified in this application are by weight unless otherwise specified.

The tungsten alloy articles of all the examples were prepared using the same procedure. A mixture of tungstic oxide, ammonium perrhenate, and nickel carbonate was thoroughly mixed in a ball mill containing ethyl alcohol. The mixed powder was then reduced in hydrogen at a temperature of between about 700° and 1,000° C. The mixed powders were then treated with a solution of paraffin wax in benzene in the conventional manner. Green compacts were formed at 15 tons per square inch pressure. The green compacts were then presintered at a temperature of between about 800° and 1,000° C. for one-half hour in a hydrogen atmosphere (dewpoint -60° F.) and were then sintered in a hydrogen atmosphere (dewpoint -60° F.) at a temperature of 1,500° C. for 1 hour. During sintering, there was a shrinkage of about 45 percent by volume of the tungsten-rhenium-nickel alloys. The metal articles produced from these alloys have unusually high density, are coherent, and have a homogeneous structure, as shown in FIG. 2, a photomicrograph (100 x) of an unetched section, and FIG. 3, a photomicrograph (425 x) of an etched section of the alloy composition 0.20 percent nickel and 3 percent rhenium.

The density of various tungsten-rhenium-nickel sintered articles is reported in table 1, together with the densities of a number of different tungsten alloys (and also unalloyed tungsten) for comparative purposes.

TABLE 1

| Example | TUNGSTEN COMPOSITIONS |      | Density (g./cc.) |
|---------|-----------------------|------|------------------|
|         | % Ni                  | % Re |                  |
| 60      |                       |      |                  |
| 1       | 0.15                  | 2    | 18.7             |
| 2       | 0.15                  | 3    | 19.0             |
| 3       | 0.15                  | 4    | 18.8             |
| 4       | 0.20                  | 0    | 18.2             |
| 5       | 0.20                  | 1    | 18.6             |
| 6       | 0.20                  | 2    | 19.2             |
| 7       | 0.20                  | 3    | 19.3             |
| 8       | 0.20                  | 4    | 19.3             |
| 9       | 0.20                  | 5    | 19.3             |
| 10      | 0.20                  | 7.5  | 18.8             |
| 11      | 0.20                  | 10   | 16.4             |
| 12      | 0.30                  | 0    | 18.1             |
| 13      | 0.30                  | 1    | 19.0             |
| 14      | 0.30                  | 2    | 19.3             |
| 15      | 0.30                  | 3    | 19.2             |
| 16      | 0.30                  | 4    | 19.2             |
| 17      | 0.30                  | 5    | 19.1             |
| 18      | 0.30                  | 7.5  | 19.2             |
| 19      | Co-0.20               | 3    | 17.5             |
| 20      | Fe-0.20               | 3    | 18.0             |

In all the compositions reported in the table, the balance of the composition was tungsten.

What is claimed is:

1. Sintered high-density tungsten alloy composition containing between about 1 and 7.5 percent rhenium, between about 0.15 and 0.3 percent nickel and the balance tungsten.

2. The compositions of claim 1 containing between about 2 and 7 percent rhenium and between about 0.2 and 0.3 percent nickel and having a density as sintered in excess of 19 g./cc.

3. The compositions of claim 1 containing about 0.3 percent nickel and having a density as sintered in excess of 19 g./cc.

4. The compositions of claim 1 containing between about 1 and 5.5 percent rhenium.

5. The compositions of claim 4 containing at least about 2 percent rhenium and containing at least about 0.2 percent nickel and having a density as sintered in excess of 19 g./cc.

6. The compositions of claim 4 containing between about 2 and 4 percent rhenium and containing about 0.15 percent nickel.

5

10

15

20

25

30

35

40

45

50

55

60

65

70

75

7. The compositions of claim 6 containing about 3 percent rhenium and having a density as sintered in excess of 19 g./cc.

8. Sintered high-density electric contacts consisting essentially of between about 1 and 7.5 percent rhenium, between about 0.15 and 0.3 percent nickel and the balance tungsten.

9. The electric contacts of claim 8 containing between about 2 and 7 percent rhenium and between about 0.2 and 0.3 percent nickel, and having a density in excess of 19 g./cc.

10. The electric contacts of claim 8 containing about 0.3 percent nickel and having a density in excess of 19 g./cc.

11. The electric contacts of claim 8 containing between 1 and 5.5 percent rhenium.

12. The electric contacts of claim 11 containing at least 2 percent rhenium and containing at least 0.2 percent nickel and having a density in excess of 19 g./cc.

13. The electric contacts of claim 11 containing between 2 and 4 percent rhenium and containing about 0.15 percent nickel.

14. The electric contacts of claim 13 containing about 3 percent rhenium and having a density in excess of 19 g./cc.

\* \* \* \* \*